# EUROPEAN PATENT SPECIFICATION

(11) **EP 3 124 634 B1**
(45) Date of publication and mention of the grant of the patent: **23.10.2024**
(21) Application number: 15183275.5
(22) Date of filing: 01.09.2015
(51) Int. Cl.: C22C 33/02, C22C 38/00, C22C 38/16, B22F 9/22, C22C 26/00

(54) **PREALLOYED IRON-BASED POWDER, A METHOD FOR THE MANUFACTURING AND USE THEREOF AND A SINTERED COMPONENT**
VORLEGIERTES AUF EISEN BASIERENDES PULVER, VERFAHREN ZU SEINER HERSTELLUNG, VERWENDUNG DAVON UND GESINTERTES TEIL
POUDRE PRÉALLIÉE À BASE DE FER, PROCÉDÉ POUR SA PRODUCTION, SON UTILISATION ET COMPOSANT FRITTE

(30) Priority: 27.07.2015 PL 41328315
(43) Date of publication of application: 01.02.2017
(73) Proprietor: Akademia Górniczo-Hutnicza im. Stanislawa Staszica w Krakowie, 30-059 Kraków (PL)
(72) Inventor: KONSTANTY, Janusz, 30-150 Kraków (PL); ROMANSKI, Andrzej, 30-611 Kraków (PL); WIECZOREK-CIUROWA, Krystyna, 30-011 Kraków (PL); SIKORA, Teodora, 31-936 Kraków (PL)
(74) Representative: Rogozinska, Alicja

(56) References cited:
- GB-A- 2 023 184
- US-A- 4 518 563
- US-A- 4 588 441
- US-B1- 6 596 224

## Description

The invention relates to an easily sinterable prealloyed iron-based powder, a method for the manufacturing and use thereof and the sintered product.

The term "easily sinterable powder" as used in present application refers to a powder that after cold forming at pressure of 100-400 MPa and free sintering (at atmospheric pressure) in a reducing atmosphere for a time no longer than 60 minutes at a temperature not higher than 950° C allows to obtain sintered parts of the total porosity of less than 5% by volume.

Factors for rendering the easily sintering nature to powders are:
- finely-crystalline structure of the powder particles, in which the polycrystalline powder particles are composed of grains having an average size of about 2 µm or less,
- two- or multi-phase structure at the sintering temperature, which, while restraining grain growth, provides finely-crystalline structure of the material during sintering,
- presence of a liquid phase during sintering.

Low-alloy iron powders containing at least 90% Fe by weight and sintered without the liquid phase allow obtaining sintered parts of the total porosity of less than 5% by volume, while maintaining the fine-grained microstructure of the material. The two-phase microstructure of the material at the sintering temperature, composed of ferrite and austenite, is assured by the chemical composition of the alloy. Ferrite stabilizers, e.g.: P, W, Mo, Co, and austenite stabilizers, e.g.: Cu, Ni, are used in quantities and proportions assessed by means of experimental techniques (e.g. the high temperature X-ray diffraction phase analysis) or analytical techniques (e.g. the ThermoCalc software^{®}) in order to obtain the ferrite-to-austenite volume ratio in the range from 2/5 to 3/5 within the possibly widest sintering temperature range. Furthermore, the increase in the phosphorus content of the powder contributes to the increase in the as-sintered hardness due to a strong solid solution strengthening effect.

The liquid phase sintered materials are characterized by a higher content of alloying elements such as Cu and Sn, which have to assure sufficient amount of persistent liquid phase at the sintering temperature in order to reach as-sintered porosity of less than 5% by volume. Liquid phase sintering of high-alloy iron powders containing at least 10% by weight of alloying elements makes it difficult to retain the fine-grained structure of the starting powder, but it promotes applicability of such powders whenever permanent bonding of the sintered part to another element must occur during sintering.

Easily sinterable iron-based powders are used for the production of sintered structural and tool products, in particular for the production of sintered metal-diamond composites obtained by the free sintering, but also by pressure sintering method. So far, the most commonly used material in these applications was a cobalt, high-alloy iron-based powders available on the market under the trade names Cobalite CNF^{®} (Umicore, Belgium) and Next 400^{®} (Eurotungstène, France) and mixtures thereof with prealloyed tin bronzes, iron, nickel and tungsten carbide (e.g.: MX4885, MX4380, MX4590, MX4940, etc.). Cobalite CNF^{®} powder is described in the publication by BJ. Kamphuis, B. Serneels: "Cobalt and nickel free bond powder for diamond tools: Cobalite CNF "Industrial Diamond Review, No. 1, 2004, pp. 26-32. These raw materials, due to the high content of expensive alloying elements and the use of chemical production methods, are expensive to manufacture. They cause a serious health hazards to the persons vulnerable to prolonged exposure to fine powders containing cobalt and/or nickel, involving the frequent occurrence of cobalt lung, giant cell interstitial pneumonia, allergic and cancerous skin diseases. The above mentioned cost and environmental factors have caused a growing tendency to reduce the content of alloying elements, especially cobalt, in easily sinterable prealloyed iron-based powders, while maintaining their required technological and functional properties. Until recently research efforts have been directed toward seeking alternatives for cobalt, i.e. replacing it with other alloying elements, in consequence of that a total content of alloying elements still remained relatively high, for example in said powders Next400 and Cobalite CNF the total content of alloying elements is 50% by weight and 31.6% by weight, respectively.

Document US 4518563 discloses a powder comprising Cr, from 2,5 to 7,5 wt.%; Mn, from 2,5 to 7,5 wt.%; P from 0.2 to 0.8 wt.%; Cu, from 1.0 to 5.0 wt.%; Si, from 0.5 to 2.0 wt.%; Mo, from 0 to 3 wt.%; C, from 1.5 to 3.5 wt.%; and the balance being Fe with less than 2 wt.% of impurities. The powder is used in a method for manufacturing an anti-wear slide member having improved anti-pitting and initial stage fit of its slide surface.

The previously known methods for manufacturing fine grain, especially easily sinterable prealloyed iron-based powders, using co-precipitation technology of metal hydroxides or oxalates from aqueous salt solutions, which, after filtration and calcination, are subjected to reduction with hydrogen, also proved unsatisfactory due to cost and environmental aspects. Such methods are known e.g. from the patent specifications US 6,554,885 B1, US 6,613,122 B1, US 6,312,497 B1, US 7,077,883 B2, EP 0 865 511 B1, EP 1 492 897 B1. Disadvantages of the known methods based on co-precipitation of hydroxides or salts are both their high cost as well as disposal problems with environmentally harmful wastes inevitable in those processes.

The object of the invention is to provide easily sinterable prealloyed iron-based powders that do not demonstrate the prior art disadvantages resulting from the high content of alloying elements. They are therefore more environmentally friendly, cheaper and easier to manufacture, while maintaining very good properties, both technological as well as functional.

The object of the invention is also to propose a method for manufacturing easily sinterable prealloyed iron-based powders, which method eliminates the disadvantages occurring in the prior art, namely it is environmentally friendly, less expensive to implement and demonstrates flexibility allowing the better adjustment of the properties of the resulting powder to a particular application.

The product of the invention is determined in independent claim 1 and dependent claims 2-3.

The easily sinterable prealloyed iron-based powder, obtained by subjecting a reducible material, successively to milling, annealing and cooling thereof and grinding the cooled material to the powder, wherein the reducible material comprising oxides, carbonates, nitrates, metals and metal alloys and mixtures thereof, reducible by a technical purity hydrogen at a temperature not higher than 750°C, wherein the powder consists of:
- at least 80% Fe by weight; alloying elements and impurities the total content of which is limited to 20% by weight and as a balance,
- wherein the alloying elements are 1-18% Cu by weight, 0.2 - 2% P by weight and 0.5 - 4% Sn by weight, and optionally
at least one alloying element as alloying additives selected from the group consisting of Co, Ni, W and Mo in the total content of Co and/or Ni and/or W and/or Mo not more than 5% by weight.

Preferably, the average particle size of the powder determined by the Fisher apparatus is not more than 10 µm.

Preferably, the powder comprises polycrystalline particles constituted of grains having average size not greater than 2 µm.

A method for producing the easily sinterable prealloyed iron-based powder according to claims 1 to 3 is determined in claims 4-7.

A method for producing the easily sinterable prealloyed iron-based powder according to claims 1 to 3, comprising the successive steps:
- preparing a reducible material comprising oxides, carbonates, nitrates, metals and metal alloys and mixtures thereof, reducible by technical purity hydrogen at a temperature not higher than 750°C;
- subjecting the said reducible material to mechanical processing by milling, including grinding, homogenization and activation of the reducible material;
- annealing the said ground homogenized and activated by milling reducible material in a reducing atmosphere;
- cooling the said reduced material to a temperature preventing its self-ignition; and
- grinding the said cooled material to a powder having a predetermined average particle size.

Preferably, the annealing is carried out at a temperature of 550-750°C, for a time of 1-8 hours, in a reducing atmosphere, which is hydrogen or a gas mixture containing hydrogen.

Preferably, the mechanical processing of the reducible material is performed in dry or wet condition.

Preferably, further drying is carried out after the mechanical processing in wet condition.

The easily sinterable prealloyed iron-based powder as described above is used for the manufacturing of sintered structural and tool components, in particular sintered metal-diamond composites.

The sintered product, especially the sintered metal-diamond composite, prepared from the easily sinterable prealloyed iron-based powder according to the invention is characterized in that the easily sinterable prealloyed iron-based powder is the powder as described above, wherein the total porosity of the sintered product at a temperature not higher than 950°C is lower than 5%.

Thus, the invention allows in a surprisingly simple and inexpensive manner to produce the easily sinterable prealloyed iron-based powder comprising at least 80% of iron by weight, copper and phosphorus, and optionally at least one from the group of alloying elements including tin, cobalt,nickel, tungsten and molybdenum, as well as impurities, mainly in the form of hardly reducible oxides such, for example SiO₂. The total content of alloying elements and impurities in the powders produced according to the invention does not exceed 20% by weight, wherein the powders in which the minimum content of alloying elements is 10% by weight are intended for applications in which it is required that permanent bonding of the sintered part to another element or elements, made of iron or its alloys, must occur during sintering, e.g. by brazing.

The easily sinterable prealloyed iron-based powder according to the invention, while maintaining properties similar to the known powders of this kind, has in comparison to them a number of economic, environmental and technological advantages such as:
- very low, limited to 20% by weight, total content of alloying elements and impurities;
- very low, limited to 5% by weight, total content of expensive, deficient and/or harmful alloying elements such as Co, Ni, W, Mo, rare earth metals, etc.;
- possibility of manufacturing sintered parts having a hardness greater than 200 HV;
- possibility of heat treatment of sintered parts and further increase in hardness above 300 HV;
- possibility of manufacturing by means of mechanochemical methods.

The method of the invention for producing the new prealloyed iron-based powders eliminates the expensive chemical method for obtaining mixtures of hydroxides, oxalates or other metal compounds hardly soluble in water, in which environmentally harmful waste (salts), that require utilization, are formed, and their later thermal decomposition to oxides occurs. It is replaced by a cheaper, mechanochemical synthesis of oxides, which, in comparison with the chemical method, gives greater freedom in selection the chemical composition of the powder. Mechanochemical synthesis consists in inducing chemical reactions preceded by grinding and mechanical activation of substrates. It enables receiving new materials characterized by a low level of chemical and structural heterogeneity, fine-grained microstructure and the most often desirable complex phase composition.

In the method according to the invention a reducible material is thus prepared through mechanical processing by milling, resulting in grinding, homogenization and activation of the reducible material. The crushed, homogenized and activated by grinding reducible material thus obtained is annealed in a reducing atmosphere, and then cooled to a temperature which prevents self-ignition of the material. Finally, the annealed and cooled material is ground to a powder having a predetermined average particle size. The application of mechanochemical processes, due to milling reagents in ball mills, simplifies synthesis procedures and eliminates the need of expensive waste utilization, which in turn significantly improves the ecology of producing high performance functional materials, thus meeting the principles of so called "Green Chemistry".

The method according to the invention has the following advantages in comparison to the traditional method of co-precipitation hydroxides or oxalates:
- environmental performance;
- lower material and equipment costs;
- possibility of flexible selection of chemical composition of the powders enabling direct influence on the properties of the final product;
- shortening the milling time due to the use of a more energetic mill.

The powders produced by the mechanochemical method of oxides synthesis are free of drawbacks, which intrinsically characterise commercial powders, while maintaining similar to them technological properties. For this reason, the presented invention has tremendous application potential.

The object of the invention is illustrated hereinafter in the embodiment and shown in the accompanying drawing, in which:
Figure 1 is a scanning electron microscope micrograph showing the structure of the powdered metal sponge obtained in Example 1;
Figure 2 is a graph obtained by X-ray diffraction phase analysis illustrating the prealloyed nature of the powder according to Example 1;
Figure 3 is a scanning electron microscope micrograph showing the structure of the powdered metal sponge obtained according to Example 3;
Figure 4 is a scanning electron microscope micrograph showing the structure of the powdered metal sponge obtained according to Example 5;
Figure 5 is the graph obtained by X-ray diffraction phase analysis illustrating the prealloyed nature of the powder according to Example 5; and
Figure 6 is a metallographic light microscope micrograph illustrating the joint between the sintered part of Example 7 and the steel substrate.

### Example 1 (reference)

A powder mixture containing 92.86 g Fe₂O₃; 3.57 g CuO and 3.57 g of prealloyed Fe-P powder containing 10% phosphorus by weight was prepared by mixing the ingredients in a Turbula type mixer for 10 minutes. The powders were placed together with grinding media in a 1.25 dm³ roller ball mill drum. 12 mm diameter 100Cr6 bearing steel balls were used as the grinding media. The degree of filling of the mill was 50% by volume, and the ball-to-powder weight ratio was 20:1. Ethyl alcohol was poured into the drum in an amount required for the complete immersion of the grinding media together with the powder in the liquid. The drum was turned on to rotate at 65% of the critical speed. After milling for 72 hours, the charge of the mill was dried in a laboratory drier at 130°C. The powder was then subjected to reducing annealing for 180 minutes at 700°C in a hydrogen atmosphere and cooled to below 30°C in order to avoid self-ignition. The thus obtained metal sponge was ground in a ceramic mortar to powder (Figure 1) with a nominal content of 95.5% Fe by weight, 4% Cu by weight and 0.5% P by weight, the hydrogen loss of 1.1% by weight and Fisher sub-sieve size of 1.3 µm. The prealloyed nature of the powder was verified by X-ray diffraction phase analysis (Figure 2).

### Example 2 (reference)

5 g portions of the powder obtained according to the procedure described in Example 1 were cold-pressed under 200 MPa in a carbide die having cavity dimensions 15.5 × 15.5 mm. The green densities of compacts was determined using the geometric method (Table 1). The powder compacts were sintered in a laboratory tube furnace for 60 minutes at 890, 900, 910, 920 and 925°C in a hydrogen atmosphere. During heating the compacts were held for 60 minutes at 700°C before proceeding to the sintering temperature. After sintering the samples were furnace cooled to room temperature. The sintered samples were tested for density by the water immersion technique (Table 1).

**Table 1**

| Green density [g/cm³] | Sintering temperature [°C] | As-sintered density [g/cm³] |
|---|---|---|
| 4.53 | 890 | 7.53 |
| 4.52 | 900 | 7.69 |
| 4.50 | 910 | 7.66 |
| 4.52 | 920 | 7.65 |
| 4.50 | 925 | 7.57 |

### Example 3 (reference)

A powder mixture containing 92.86 g Fe₂O₃; 3.57 g CuO and 3.57 g of prealloyed Fe-P powder containing 10% phosphorus by weight was prepared by mixing the ingredients in a Turbula type mixer for 10 minutes. The powders were placed together with grinding media in a 1.25 dm³ roller ball mill drum. 12 mm diameter 100Cr6 bearing steel balls were used as the grinding media. The degree of filling of the mill was 50% by volume, and the ball-to-powder weight ratio was 20:1. Distilled water was poured into the drum in an amount required for the complete immersion of the grinding media together with the powder in the liquid. The drum was turned on to rotate at 65% of the critical speed. After milling for 24 hours, the charge of the mill was dried in a laboratory drier at 130°C. The powder was then subjected to reducing annealing for 180 minutes at 700°C in a hydrogen atmosphere. After cooling to below 30°C the obtained metal sponge was ground in a ceramic mortar to powder (Figure 3) with a nominal content of 95.5% Fe by weight, 4% Cu by weight and 0.5% P by weight, the hydrogen loss of 1.2% by weight and Fisher sub-sieve size of 2.15 µm.

### Example 4 (reference)

5 g portions of the powder obtained according to the procedure described in Example 3 were cold-pressed under 200 MPa in a carbide die having cavity dimensions 15.5x15.5 mm. The green densities of compacts was determined using the geometric method (Table 2). The power compacts were sintered in a laboratory tube furnace for 60 minutes at 900°C in a hydrogen atmosphere. During heating the compacts were held for 60 minutes at 700°C before proceeding to the sintering temperature. After sintering the samples were furnace cooled to room temperature. The sintered samples were tested for density by the water immersion technique (Table 2). Selected sintered samples were then solution treated by reheating to 900°C, holding for 30 minutes in nitrogen and quenching in water. Then they were aged for 60 minutes at 400, 450, 475, 500, 550 and 600°C. The sintered parts were tested for a Vickers hardness determined at a 1 kgf load (Table 2).

**Table 2**

| Green density [g/cm³] | As-sintered density [g/cm³] | Variant of the heat treatment | HV1 ⁽¹⁾ |
|---|---|---|---|
| 4.63 | 7.74 | as-sintered condition | 212 ± 5 |
| 4.63 | 7.74 | solution treated | 209 ± 7 |
| 4.65 | 7.71 | solution treated and aged at 400°C | 228 ± 7 |
| 4.66 | 7.72 | solution treated and aged at 450°C | 297 ± 10 |
| 4.64 | 7.72 | solution treated and aged at 475°C | 312 ± 8 |
| 4.65 | 7.71 | solution treated and aged at 500°C | 304 ± 8 |
| 4.64 | 7.72 | solution treated and aged at 550°C | 286 ± 6 |
| 4.66 | 7.72 | solution treated and aged at 600°C | 240 ± 11 |

| | | | |
|---|---|---|---|
| ⁽¹⁾ The confidence intervals were estimated for a confidence level 1-α = 0.9 | | | |

### Example 5

10 g of dry powder mixture comprising 8.82 g Fe₂O₃; 0.68 g CuO; 0.36 g of prealloyed Fe-P powder containing 10% phosphorus by weight and 0.14 g Sn was placed together with 100 g of 10 mm diameter steel balls in a 0.25 dm³ steel reactor of a laboratory, planetary ball mill (Activator 2S, Novosibirsk Corp.). The charge was then subjected to high-energy milling for 2 hours at a rotational speed of 700 rpm in air atmosphere. During the milling process the reactor was water-cooled. In this manner, the composite oxide powder having a modified crystalline microstructure and characterized by a high susceptibility to reduction in hydrogen was obtained. The powder was then subjected to reducing annealing for 180 minutes at 700°C in a hydrogen atmosphere and cooled to below 30°C in order to avoid self-ignition. The metal sponge thus obtained was ground in a ceramic mortar to a powder (Figure 4) with a nominal content of 90% Fe by weight, 7.5% Cu by weight, 2% Sn by weight and 0.5% P by weight, the hydrogen loss of 0.6% by weight and Fisher sub-sieve size of 8 µm. The prealloyed nature of the powder was verified by X-ray diffraction phase analysis (Figure 5).

### Example 6

5 g portions of the powder obtained according to the procedure described in Example 5 were cold-pressed under 200 MPa, in a carbide die having cavity dimensions 15.5x15.5 mm. The green densities of compacts was determined using the geometric method (Table 3). The powder compacts were sintered in a laboratory tube furnace for 60 minutes at a temperature 900°C in a hydrogen atmosphere. During heating the compacts were held for 60 minutes at 700°C before proceeding to the sintering temperature. After sintering the samples were furnace cooled to room temperature. The sintered parts were tested for density by the water immersion technique (Table 1) and for Vickers hardness determined at a 1 kgf load (Table 3).

**Table 3**

| Green density [g/cm³] | As-sintered density [g/cm³] | HV1 ⁽¹⁾ |
|---|---|---|
| 4.57 | 7.94 | 230 ± 8 |

| | | |
|---|---|---|
| ⁽¹⁾ The confidence intervals were estimated for a confidence level 1- α = 0.9 | | |

### Example 7

5 g portions of the powder obtained according to the procedure described in Example 5 were cold-pressed under 200 MPa in a carbide die having cavity dimensions 15.5×15.5 mm. The green compacts were placed on a plain low-carbon steel sheet and sintered in a laboratory tube furnace for 60 minutes at 900°C in a hydrogen atmosphere. During heating the compacts were held for 60 minutes at 700°C before proceeding to the sintering temperature. After sintering the samples were furnace cooled to room temperature. After sintering, metallographic specimens were prepared to make a qualitative evaluation of the joint between the sintered part and the steel substrate. A light microscope was used to the analysis (Figure 6).

## Claims

1. An easily sinterable prealloyed iron-based powder, wherein the powder consists of:
- at least 80% Fe by weight,
- alloying elements and impurities the total content of which is limited to 20% by weight and as a balance,
- wherein the alloying elements are 1-18% Cu by weight, 0.2 - 2% P by weight and 0.5 - 4% Sn by weight, and optionally
- at least one alloying element as alloying additives selected from the group consisting of Co, Ni, W and Mo in the total content of Co and/or Ni and/or W and/or Mo not more than 5% by weight.

2. The easily sinterable prealloyed iron-based powder according to claim 1, **characterized in that** average particle size of the powder, determined by the Fisher apparatus, is not more than 10 µm.

3. The easily sinterable prealloyed iron-based powder according to any one of the preceding claims, **characterized in that** the powder comprises polycrystalline particles containing grains having average size not greater than 2 µm.

4. A method for producing the easily sinterable prealloyed iron-based powder according to claims 1 to 3, comprising the successive steps:
- preparing a reducible material comprising oxides, carbonates, nitrates, metals and metal alloys and mixtures thereof, reducible by a technical purity hydrogen at a temperature not higher than 750°C;
- subjecting the said reducible material to mechanical processing by milling, including grinding, homogenization and activation of the reducible material;
- annealing the said ground homogenized and activated by milling reducible material in a reducing atmosphere;
- cooling the said annealed material to a temperature preventing its self-ignition; and
- grinding the said cooled material to a powder having a predetermined average particle size.

5. The method according to claim 4, **characterized in that** the annealing is carried out at a temperature of 550-750°C, for a time of 1- 8 hours, in a reducing atmosphere, which is hydrogen or gas mixture containing hydrogen.

6. The method according to claims 4 or 5, **characterized in that** the mechanical processing of the reducible material is performed in dry or wet condition.

7. The method according to claim 4, **characterized in that** further drying is carried out after the mechanical processing in wet condition.

8. Use of the easily sinterable prealloyed iron-based powder according to any one of the claims 1 to 3 for the manufacturing of sintered structural and tool components, in particular sintered metal-diamond composites.

## Patentansprüche

1. Leicht sinterbares vorlegiertes Pulver auf Eisenbasis, wobei das Pulver
- mindestens 80 Gew.-*%* Fe;
- Legierungselemente und Verunreinigungen, deren Gesamtgehalt zu 20 Gew.% und als Rest begrenzt ist;
- wobei die Legierungselemente 1-18 Gew.-% Cu, 0,2-2 Gew.-% P und 0,5 bis 4 Gew.-% Sn sind, und wahlweise
- mindestens ein Legierungselement aus der Co, Ni, W und Mo enthaltenden Gruppe, wobei der Gesamtgehalt an Co und/oder Ni und/oder W und/oder Mo nicht mehr als 5 Gew.-% beträgt,
enthält.

2. Leicht sinterbares vorlegiertes Pulver auf Eisenbasis nach Anspruch 1, **dadurch gekennzeichnet, dass** die durchschnittliche Partikelgröße des Pulvers, bestimmt mit dem Fisher-Gerät, nicht mehr als 10 um beträgt.

3. Leicht sinterbares vorlegiertes Pulver auf Eisenbasis nach einem der vorherigen Ansprüche, **dadurch gekennzeichnet, dass** das Pulver polykristalline Partikel enthält, deren Körner eine durchschnittliche Größe von nicht mehr als 2 µm aufweisen.

4. Verfahren zur Herstellung des leicht sinterbaren vorlegierten Pulvers auf Eisenbasis nach den Ansprüchen 1 bis 3, umfassend nachfolgende Schritte:
- Bereitstellen eines reduzierbaren Materials, umfassend Oxide, Carbonate, Nitrate, Metalle und Metalllegierungen und Mischungen davon, reduzierbar mit dem technischen Wasserstoff bei einer Temperatur von nicht mehr als 750°C.
- mechanische Verarbeitung des reduzierbaren Materials durch Mahlen, einschließlich Zerkleinern, Homogenisieren und Aktivieren des reduzierbaren Materials;
- Glühen des zerkleinerten homogenisierten und durch Mahlen aktivierten reduzierbaren Materials in einer reduzierenden Atmosphäre;
- Kühlen des geglühten Materials auf eine Temperatur, die seine Selbstzündung verhindert; und
- Zerkleinern des gekühlten Materials zu einem Pulver mit einer vorgegebenen mittleren Partikelgröße.

5. Verfahren nach Anspruch 4, **dadurch gekennzeichnet, dass** das Glühen bei einer Temperatur von 550-750°C für eine Zeit von 1-8 Stunden in einer reduzierenden Atmosphäre durchgeführt wird, wobei die reduzierende Atmosphäre Wasserstoff oder ein Wasserstoff enthaltendes Gasgemisch ist.

6. Verfahren nach Anspruch 4 oder 5, **dadurch gekennzeichnet, dass** die mechanische Verarbeitung des reduzierbaren Materials eine Trockenverarbeitung oder eine Nassverarbeitung ist.

7. Verfahren nach Anspruch 4, **dadurch gekennzeichnet, dass** nach der mechanischen Nassverarbeitung eine weitere Trocknung durchgeführt wird.

8. Verwendung des leicht sinterbaren vorlegierten Pulvers auf Eisenbasis nach einem der Ansprüche 1 bis 3 zur Herstellung von gesinterten Bau- und Werkzeugteilen, insbesondere von gesinterten Metall-Diamant-Verbundmaterialien.

## Revendications

1. Poudre alliée facilement frittable à base de fer, laquelle contient
au moins 80% en poids de Fe,
des éléments d'addition et des impuretés, dont la teneur totale est limitée à 20% en poids et en tant que complément,
les éléments d'addition représentant 1-18*%* en poids de Cu, 0,2-2*%* en poids de P et 0,5-4*%* en poids de Sn, et optionnellement
au moins un élément d'addition comme addition choisi dans le groupe contenant Co, Ni, W et Mo, où la teneur totale de Co et/ou Ni et/ou W et/ou Mo n'est pas supérieure à 5% en poids.

2. Poudre alliée facilement frittable à base de fer selon la revendication 1, **caractérisée en ce que** la grandeur moyenne des graines constituant des particules polycristallines de la poudre, déterminée au moyen de l'appareil de Fisher, n'est pas supérieure à 2 µm.

3. Poudre alliée facilement frittable à base de fer selon l'une quelconque des revendications précédentes, **caractérisée en ce que** la poudre contient des particules polycristallines de grandeur moyenne des graines ne dépassant pas les 2 µm.

4. Procédé de production de poudre alliée facilement frittable à base de fer selon l'une des revendications 1 à 3, comprenant les étapes suivantes:
préparation d'un matériau réductible, comprenant des oxydes, des carbonates, des nitrates, des métaux et alliages métalliques ainsi que leurs mélanges, réductibles avec de l'hydrogène dans une température ne dépassant pas les 750°C;
soumettre ledit matériau réductible à un traitement mécanique par broyage, comprenant le concassage, la homogénéisation et l'activation du matériau réductible;
recuit dudit matériau réductible concassé, homogénéisé et activé par broyage du matériau réductible dans une atmosphère réductrice;
refroidissement dudit matériau recuit jusqu'à une température rendant impossible son autoallumage; et
concassage dudit matériau refroidi pour obtenir une poudre d'une grandeur consignée des particules.

5. Procédé selon la revendication 4, **caractérisé en ce que** le recuit est réalisé dans une température de 550-750°C, pendant 1-8 heures, dans une atmosphère réductrice constituée par l'hydrogène ou un mélange des gaz contenant de l'hydrogène.

6. Procédé selon la revendication 4 ou 5, **caractérisé en ce que** le traitement mécanique du matériau réductible est un traitement sec ou humide.

7. Procédé selon la revendication 4, **caractérisé en ce que** après le traitement mécanique humide on procède au séchage.

8. Utilisation de poudre alliée facilement frittable à base de fer selon l'une des revendications 1 à 3 pour la réalisation des alliages frittés structurels et d'outillage, notamment des alliages frittés composites diamant-métal.
